

Dec. 22, 1953

C. S. MILLER ET AL

2,663,657

HEAT-SENSITIVE COPYING PAPER

Filed May 15, 1952

2 Sheets-Sheet 1



Inventors  
Carl S. Miller  
By Bryce L. Clark  
Carpenter, Abbott, Coulter, & Kinney  
Attorneys

Dec. 22, 1953

C. S. MILLER ET AL

2,663,657

HEAT-SENSITIVE COPYING PAPER

Filed May 15, 1952

2 Sheets-Sheet 2

Fig. 5



Inventors  
Carl S. Miller  
Bryce L. Clark  
By  
Carpenter, Abbott, Coulter & Kinney  
Attorneys

## UNITED STATES PATENT OFFICE

2,663,657

## HEAT-SENSITIVE COPYING PAPER

Carl S. Miller and Bryce L. Clark, St. Paul, Minn.,  
assignors to Minnesota Mining & Manufacturing Company, St. Paul, Minn., a corporation of Delaware

Application May 15, 1952, Serial No. 288,006

12 Claims. (Cl. 117—36)

This invention is concerned with duplicator sheet material or copying-paper useful in preparing copies of printed matter of the like, and with compositions and methods related thereto. The invention particularly contemplates heat-sensitive coatings and coated sheet materials of a novel type, and methods of utilizing such materials in preparing duplicate copies of printed or other graphic subject-matter by simple exposure to high intensity irradiation and without subsequent developing or fixing operations.

This application is a continuation-in-part of our copending application Serial No. 747,339, filed May 10, 1947.

Prior art copying-papers of which we are aware, which are subjected to exposure to visible light or similar forms of radiant energy in the preparation of copies of graphic subject-matter, must be protected from light before use, and require various processing steps, in addition to the initial controlled exposure, for the production of visible light-stable copies.

Our new heat-sensitive copying-paper, on the contrary, is not itself affected by radiant energy such as visible or ultra-violet light, and may therefore be left exposed to such radiations both before and after printing. Nevertheless, radiant energy may be employed as the sole agency for the production of visible light-stable and permanent copies of graphic subject-matter on our novel copying-paper, or on other surfaces carrying our novel heat-sensitive compositions, by processes as hereinafter set forth.

The processes by which we are enabled to achieve this result, e. g. in the preparation of copies of the printed pages of books or the like, involve the irradiation of the printed surface, the resultant formation of an elevated-temperature pattern corresponding to the graphic subject-matter of such printed surface, and the utilization of this elevated-temperature pattern in the development of a facsimile copy of the graphic subject-matter on the heat-sensitive copying-paper.

Formulas may be found in the prior art for various heat-sensitive paints, coated sheet materials, and the like. All such products of which we are aware exhibit one or more significant deficiencies when compared with our novel heat-sensitive compositions and coated products. They may be sensitive to light as well as heat. They may require an extremely high temperature, or a relatively long time at a specific temperature, or heating over a wide range of temperature, to produce a visible change of sufficient intensity,

5 The change obtained at elevated temperatures may be reversible on cooling, i. e. the product exhibits thermotropy. These and other deficiencies of prior art materials are avoided by the use of our novel compositions and products, particularly in connection with the copying of printed matter such as books, drawings or diagrams, pictures, etc. by means of our novel copying-paper herein described and illustrated.

10 The heat-sensitive compositions of our invention are comprised of solid ionizable reactants of which at least one is an electron donor component and another an electron acceptor component, which are potentially chemically capable of irreversibly and rapidly reacting at normal room temperature in a direct ion-exchange electron acceptor-donor chemical reaction to produce a visibly different reaction product, but which are normally maintained in physically distinct relationship and physically prevented from so reacting. 15 The structure is so designed that an increase in temperature to a predetermined level allows the reaction to take place. The reaction is believed to be initiated by the melting, or softening, or other physical change, of one or more of the reactive substances. Whatever the specific physical change employed, the application of heat results in an immediate reaction of the reactants and formation of a colored, opaque, or otherwise visibly different reaction product.

20 The rapid rate of reaction obtainable by this means is particularly advantageous where the reactive material in sheet form is to be used as a heat-sensitive copying-paper. For the most effective reproduction of drawings or the like containing fine lines as well as massive dark areas, a high contrast number, as hereinafter defined, must be obtained when the sheet is heated through a narrow range of temperature not greater than about 20° C. and preferably about 5° C., within a period of time not greater than one second, and preferably within about one-tenth of a second, in order to obtain desirable contrast and detail.

25 40 45 Where these limitations are exceeded, the reproductions obtained may be blurred, "fuzzy," or otherwise of poor quality. For example, a heat-sensitive sheet material which darkens over a wide range of temperature, e. g. which provides a contrast number of 0.2 when heated to 70° C. but does not reach a contrast number of 0.8 until heated to 110° C., will ordinarily not produce a print having good contrast between light and dark areas.

50 55 A convenient method of determining the rate

of reaction as well as the required temperature of activation for a particular copying-paper involves placing portions of the sheet against a series of metal surfaces each at a different but controlled temperature, and for various intervals of time. Our preferred copying-papers, when so tested, show a reaction from the original state to a color intensity or opacity equivalent to a contrast number of at least about 0.4, and preferably about 0.9, when heated at the required temperature level and within a temperature range of not more than about 20° C., and within a contact time of not more than about one-tenth second.

In determining the contrast number of a copying-paper, suitably exposed samples having printed (darkened) and unprinted (undarkened) areas are held against a flat magnesium carbonate block (a "standard magnesium carbonate surface" as defined in the paint industry). A beam of white light (north exposure daylight) is directed against the outer surface of the sample at an angle of 45°, and the intensity of the light reflected normal to the surface is measured by means of a suitable photometer. The contrast number is defined as the following ratio.

$$\frac{I_u - I_d}{I_u}$$

where  $I$  represents intensity, and subscripts  $u$  and  $d$  refer to measurements made over the undarkened area and darkened area, respectively.

The following examples of specific compositions and structures will serve more clearly to point out and explain the novel concept here involved, but are not to be construed as limitative.

#### EXAMPLE 1

*Reactant A.*—To an aqueous solution of three mols of the sodium soap of commercial triple-pressed stearic acid of melting-point approximately 53° C., and which supposedly contains a minor amount of other higher fatty acids, etc., add an aqueous solution of one mol of ferric sulfate. Filter the precipitated ferric stearate, wash separately with water and alcohol, and dry at room temperature. The solid product softens or melts within the range of 70–95° C. Disperse 500 grams of the powder in two liters of denatured ethyl alcohol, e. g. "Ponsolve," by grinding with flint pebbles in a ball mill.

*Reactant B.*—Dissolve 1500 grams of hexamethylenetetramine in 12 liters of denatured alcohol ("Ponsolve") at 65° C.; with constant stirring, add this solution to a solution of 2000 grams of pyrogallic acid in 4 liters of the alcohol, also at 65° C. A crystalline precipitate forms. Cool to room temperature, with constant stirring to avoid lumping. Recover and dry the precipitate, which should be in the form of a fine powder. Disperse 500 grams of this powder in one and one-half liters of denatured alcohol by ball milling as for reactant A.

*Reactant C.*—Dissolve 10 grams of oxalic acid in 100 milliliters of ethyl alcohol.

*Binder.*—Dissolve 150 grams of polyvinyl butyral in one liter of ethyl alcohol.

#### Composition in liquid form

|                       | ML. |
|-----------------------|-----|
| Reactant A            | 500 |
| Reactant B            | 100 |
| Reactant C (optional) | 40  |
| Binder                | 200 |

In mixing and temporarily maintaining the mixture of reactants A and B in a volatile ve-

hicle such as denatured ethyl alcohol, a slight discoloration may sometimes be noted. This is presumably due to solution of traces of one or both of the substantially insoluble reactants in the liquid vehicle and the resultant reaction of the dissolved materials to produce a dark-colored reaction product. The presence of a trace of oxalic acid, which forms a complex with iron and consequently may be considered to render inaccessible any dissolved or previously reacted iron, discharges and/or prevents the formation of the slight discoloration thus otherwise produced. Citric acid, which likewise forms an iron complex, is also effective. In many cases the discoloration produced, even in the absence of these modifying reactants, is so slight as not to be troublesome, particularly where adequate precautions are taken in preparing and in applying the temperature-sensitive composition.

#### Coated transparent sheet material

The above liquid composition is uniformly spread, as by means of a spreader bar or knife coater, over one surface of a thin transparent film of plasticized regenerated cellulose (cellophane) to a thickness of approximately 3 mils, and is allowed to dry at room temperature. The resulting visibly transparent coated sheet product rapidly darkens when heated to or above about 80° C., and is suitable for use as a temperature-sensitive copying-paper.

The darkening here obtained is thought to result from a preliminary melting or softening of the ferric stearate, making possible the mixing or co-dissolving of the two reactants and their resulting rapid reaction to form a dark-colored and opaque reaction product. This may be inferred from the fact that the darkening of the sheet is obtained on heating the copying-paper to a temperature closely approximating the melting or softening point of the particular ferric soap used. A similar color change may be produced at room temperature by adding a suitable solvent, e. g. benzol, to the otherwise non-reacting mixture of the two powders.

This reaction and rapid color change does not take place on exposure of the mixture, or of the coated sheet material, to radiant energy such as visible or infra-red light in the absence of the required temperature increase. Some darkening of the coated transparent sheet material as above prepared may be observed on prolonged exposure to light, and particularly to high intensities of actinic radiation; but this is believed to be due to the effect of certain radiations decomposing one or both of the reactants separately, and may readily be prevented by applying a suitable filter over the temperature-sensitive coating. A thin surface coating of a mixture of 3 grams of 4,4'-dihydroxy-benzalazine and 15 grams of polyvinyl butyral, applies from solution in 85 grams of alcohol, provides an effective filter for this purpose.

#### EXAMPLE 2

To obtain a composition having improved aging characteristics and which will react when heated to a somewhat lower temperature, similarly prepared ferric myristate, made with commercial myristic acid, is substituted for the ferric stearate of Example 1, and a reaction product of hexamethylenetetramine and gallic acid (a substituted trihydroxy benzene) is substituted for the pyrogallic acid product there described.

This second ingredient is prepared as follows: 280 grams of hexamethylenetetramine are dissolved in one liter of water, and 188 grams of gallic acid are dissolved in one liter of ethyl alcohol. One volume of the first solution is mixed with two volumes of the second, and the resulting precipitate is then recovered and dried. It is ground into heptane, by means of a ball mill, to form a 25% dispersion.

Ferric myristate softens and melts at somewhat lower temperatures than the stearate. Since the myristate is somewhat soluble in alcohol, heptane is used as the liquid vehicle, which necessitates the substitution, for the alcohol-soluble but heptane-insoluble polyvinyl butyral, of a heptane-soluble binder. In a specific example, natural rubber was used as the binder. Heptane is substantially a non-solvent for both ferric myristate and the reaction product of hexamethylenetetramine and gallic acid. There is ordinarily no visible evidence of reaction of the two materials in freshly prepared mixtures in heptane, although reaction takes place rapidly at temperatures below that required for activation of the coated copying-paper, and usually at or even below normal room temperatures, as in the case of the reactants of Example 1, in the presence of a suitable solvent such as benzene. The final composition of the fluid mass prepared according to the above description and ready for coating is approximately as follows:

| Parts by weight                                     |     |
|-----------------------------------------------------|-----|
| Ferric myristate                                    | 100 |
| Hexamethylenetetramine-gallic acid reaction product | 25  |
| Rubber                                              | 25  |
| Heptane                                             | 500 |

This composition was coated on a thin paper, i. e. an unfilled flax paper of one mil thickness, such as is used for cigarette-paper. The mixture was applied by means of a knife-coater set to give a coating orifice of approximately 3 mils, and was dried at room temperature. The coated and at least partially impregnated sheet product was faintly tan in color and appeared semi-transparent. On heating to about 70° C. it rapidly darkened and became opaque. Exposure to light alone had substantially no effect on the appearance of the unheated material. Scribing or otherwise mechanically compacting or disrupting the surface coating did not initiate the color-developing reaction.

For improved permanence, the rubber used as binder may be protected, as by the addition of suitable antioxidants or other age-resistors; or various synthetic polymers or resins may be substituted for natural rubber where their properties, e. g. color, permanence, etc., permit or encourage such substitution.

A particularly desirable copying-paper, capable of rapidly producing a high contrast ratio when heated within a range of only 5° C., was produced by employing the hexamethylene tetramine-gallic acid reaction product in conjunction with ferric stearate prepared from highly purified stearic acid.

#### EXAMPLE 3

Ferric stearate in 5 times its weight of stearic acid was emulsified in a hot concentrated solution of glue in water. To the cooled solution was added a water solution of tannic acid. The resulting well-mixed composition was coated on paper and dried at room temperature. The sheet was red-

dish-brown, but turned black when heated as in the preparation of copies of graphic subject-matter by our novel method.

#### EXAMPLE 4

Ferric stearate was dispersed in acetone by ball milling as in the previous examples, and a pre-formed solution of ethyl cellulose was added, to a final formula of approximately 12% ferric stearate, 6% ethyl cellulose, and 82% acetone. The mixture was coated in a thin uniform layer on one mil condenser tissue, a thin, tough paper, and dried at room temperature. The weight of the dry coating of ferric stearate particles uniformly dispersed in ethyl cellulose was about 0.68 gram per square foot of surface.

Gallic acid, which is a solid at normal room temperature, was dissolved in an acetone solution of ethyl cellulose, to a final formula of approximately 5% gallic acid, 9.5% ethyl cellulose, and 85.5% acetone. This solution was coated in a thin layer over the dry ferric stearate-ethyl cellulose layer, and the sheet again dried at room temperature. The dry weight of the second coating was about 0.05 gram per square foot.

The completed sheet material was useful as a copying-paper, showing high contrast and good detail in the copy. The ferric stearate component softens or melts at 70-95° C., and at least the major portion of the color change in the copy-sheet occurs over substantially the same temperature range.

#### EXAMPLE 5

35 Fifty parts by weight of ferric stearate were dispersed in 1500 parts of acetone by ball milling. Separately, 100 parts of a phenolic resin were dispersed in 400 parts of acetone by similar procedure. The phenolic resin was a solid heat-advancing partial reaction product of para-tertiary-butylphenol and formaldehyde, melting at 144-158° F. (62-72° C.). Such a resin is soluble in drying oils and aromatic hydrocarbons but insoluble in alcohols and only slightly soluble in acetone.

50 Two parts of the ferric stearate dispersion were mixed with one part of the resin dispersion, and the mixture was coated on thin paper and dried at room temperature. The resulting sheet material was useful as a heat-sensitive copying-paper, but the heat-sensitive coating had a tendency to stick to contacting surfaces, particularly during the copying process. Substitution of a higher-melting heat-advancing phenolic resin for the resin hereinbefore described eliminates this tendency, resins melting above 120° C. providing fully non-sticking surfaces with, however, some reduction in contrast in the copy obtained. Sticking is also readily avoided, and with no significant reduction in contrast, by incorporating small amounts of a film-forming binder, such as ethyl cellulose, in the mixture prior to coating.

65 Other combinations of solid visibly inter-reactive materials which have provided effective heat-sensitive copying-papers when coated on various paper or film backings in the form of dispersions in solutions of film-forming binders include ferric stearate-triethyl sulfonium tannate; ferric stearate-cadmium tannate; and ferric stearate-ammonium salicylate. Ferric myristate, ferric palmitate, and similar salts of other organic acids softening or melting at temperatures within the range of about 60-120° C. may be substituted for the ferric stearate in these compositions.

In these examples, the visible change obtained on activation of the coated material is the result of a combination between the iron of the ferric stearate or equivalent and the phenolic portion of pyrogallol or gallic acid, tannates, salicylates, or the like. A large number of other phenols which similarly provide colored reaction products with iron salt are listed by Wess and Brode in the Journal of the American Chemical Society, volume 56, at pages 1039 and 1040.

## EXAMPLE 6

One pound of nickel acetate (tetrahydrate) was dispersed in one liter of anhydrous butyl acetate by grinding in a ball mill. Similarly, one pound of calcium sulfide was ground into one liter of anhydrous butyl acetate. A 30% solution of  $\frac{1}{2}$  second nitrocellulose in butyl acetate and benzol was used as the binder. The three components were proportioned as follows:

|                            | Volumes |
|----------------------------|---------|
| Nickel acetate dispersion  | 20      |
| Calcium sulfide dispersion | 5       |
| Binder                     | 30      |

This mixture was applied in a thin layer to various supporting surfaces, e. g. cellophane or cellulose acetate film, paper, wood, leather, etc., and dried at room temperature. The dried film was faintly greenish-white in appearance. When heated, the film rapidly became intensely black and opaque.

The reactive ingredients of Example 6 are found to be inter-reactive under proper conditions at normal room temperature, with the production of a dark-colored and opaque reaction product. For example, the addition of a small amount of water to a mixture of nickel acetate and calcium sulfide in powder form initiates the reaction between the two compounds. It is believed that the reaction obtained in the coated sheet material is due to the increased vapor pressure, at an elevated temperature, of the water present in the hydrated salt, and/or the melting of the hydrous salt to a fluid state, resulting in a reactive mingling of the nickel compound and the sulfide.

## EXAMPLE 7

Strontium sulfide and nickel acetate tetrahydrate were ground up in a 21% solution of 5-second nitrocellulose in butyl acetate, in the ratio of one gram each of insoluble strontium sulfide and nickel acetate tetrahydrate particles to three milliliters of nitrocellulose solution. The mixture was coated on cellophane and dried at room temperature. The sheet was light gray in color, changing to an intense black when briefly heated to 115° C. It could be used as a heat-sensitive copying-sheet by methods described herein, producing copies of good contrast and detail.

Barium sulfide and nickel acetate tetrahydrate produce similar results. In a specific formulation, 20 ml. of a dispersion of one pound of the nickel acetate in 1000 ml. of butyl acetate, 50 ml. of a 28% nitrocellulose solution in butyl acetate, and 10 ml. of a dispersion of one pound of barium sulfide in 1000 ml. of butyl acetate were mixed and coated on paper, and dried at room temperature. A protective surface sizing of a 15% solution of nitrocellulose in butyl acetate was applied over the heat-sensitive coating and dried. The finished copying-sheet was light yellowish green in color, and produced dark-colored brown-black copies when used as a heat-sensitive copying-paper by methods above indicated. Tested on a

metal test block, the visible reaction was found to occur at approximately 93-105° C.

Other film-forming cellulose derivatives, as well as various non-cellulosic binders such as polyvinyl butyral, rubber, polyvinyl acetate, rubber hydrochloride and the like, may be substituted for the specific binder above mentioned, provided the volatile solvents required for such binders are at the same time non-solvents for, and non-reactive with the particulate solid components.

## EXAMPLE 8

Another combination of heavy metal salt and alkaline earth metal sulfide which has produced useful copies when employed in structures such as that of Examples 6 and 7 contains solid particles of nickel stearate and barium sulfide in a nitrocellulose binder. The nickel stearate, prepared by precipitation from a mixture of aqueous solutions of nickel acetate and the sodium salt of commercial stearic acid, is a waxy solid at temperatures below 60° C., and liquid at 120° C. The coated and dried sheet was dipped into a 4:1 blend of naphtha and mineral oil and again dried; the residual mineral oil improved the heat-conductivity properties of the sheet. On a metal test block, the sheet changed rapidly from light yellow to dark brown at about 113° C.; it could be used in making effective facsimile copies of typewritten letters and the like by the methods herein described.

## EXAMPLE 9

The reaction of Example 8 can be obtained at a lower temperature by incorporating in the heat-sensitive film a small proportion of a free organic acid. The following combinations of reactants, suspended in particulate form in a 5% solution of crepe rubber in heptane, coated on flax paper, and dried at room temperatures, were each effective as heat-sensitive copying-papers and produced the indicated color change at the temperature specified.

1. Nickel palmitate — barium sulfide — stearic acid; changed from light green to intense black at 85° C. Calcium sulfide produced a light gray sheet with otherwise identical properties.
2. Nickel palmitate — barium sulfide — palmitic acid; changed from light gray to intense black at 70° C.
3. Nickel caprylate — calcium sulfide — stearic acid; changed from gray to intense black at 60° C. Crotonic acid in place of stearic acid raised the conversion temperature to 72° C.
4. Many other compounds in addition to the several materials previously enumerated have additionally been found to produce adequate color differences when combined as closely spaced particles in a film-forming binder as described in the above Examples 6-9. Cobalt and lead salts are, for example, equally as effective as the salts of nickel. Salts of silver, mercury, copper and iron are useful but less desirable, silver and mercury salts showing a tendency to darken on exposure of the paper to sunlight and copper and iron salts being initially undesirably dark in color and hence providing less contrast in the resulting copy. Colorless or lightly colored sulfides such as zinc sulfide, cadmium sulfide, and magnesium sulfide are effective in formulations such as those of Example 9 and for such purposes may be considered fully equivalent to the alkaline earth metal sulfides specified in that example.

## EXAMPLE 10

Commercial octadecyl amine was dissolved as the soluble hydrochloride by heating in water and adding hydrochloric acid until the oily material was dissolved. To this was added a saturated aqueous solution of potassium ferrocyanide. The yellowish precipitate of octadecyl ferrocyanide formed by this procedure was recovered, washed, dried, and dispersed in a nitrocellulose lacquer in a mixture of butyl acetate and toluene. Twice this amount of ferric stearate, prepared as described in connection with Example 1, was separately dispersed in a portion of the lacquer. The nitrocellulose amounted to about one-fourth the total weight of the ferric stearate and the octadecyl ferrocyanide when the two dispersions were mixed.

The mixture was coated on thin paper and dried at room temperature. The coated sheet was light gray, becoming dark blue when heated to about 80° C., and producing clear and distinct thermocopies of typewritten letters and the like.

A somewhat similar product was prepared with dispersions, in an alcohol solution containing polyvinyl butyral binder and a small amount of benzoic acid, of ferric stearate and of the alcohol-insoluble reaction product of octyl amine and potassium ferricyanide. The dried coated sheet was light yellowish green in color, changing to an intense blue when heated to about 90° C.

## EXAMPLE 11

Lead myristate was prepared by adding an aqueous solution of lead acetate to an aqueous solution of the sodium soap of commercial myristic acid. The washed and dried product was dispersed in three times its weight of heptane by ball milling with flint balls. A dispersion of S-diphenyl carbazole in four times its weight of heptane was separately similarly prepared. Twenty parts by weight of each dispersion was mixed together, and 5 parts of a 30% solution of rubber hydrochloride ("Pliolite") added. The mixture was coated on condenser-tissue and dried at room temperature. The dried sheet was white in appearance, quickly changing to scarlet when heated to approximately 85-90° C. It was useful as a heat-sensitive copying-paper.

## EXAMPLE 12

A dispersion was prepared, by ball milling, of 100 parts by weight of cadmium stearate in 500 parts of heptane. The cadmium stearate was prepared by precipitation from a solution of the sodium soap of triple-pressed stearic acid. Separately, a dispersion of 20 parts of diphenyl carbazole in 200 parts of heptane, and a solution of 10 parts of crepe rubber in 90 parts of heptane, were provided. The two dispersions and the solution were mixed in the weight ratio of 1:2:3 to provide a liquid mixture which was coated onto flax tissue and dried at room temperature. The sheet was yellowish tan, rapidly changing to red at approximately 100° C., and served as a useful heat-sensitive copying-paper.

## EXAMPLE 13

Mercuric stearate was submitted for the cadmium stearate and S-diphenyl carbazine for the diphenyl carbazole of Example 12, the remaining ingredients and the relative proportions remaining the same. The coated sheet was light gray, changing rapidly to purple when heated to approximately 90° C., and could be used to

provide copies of printed matter by thermocopying methods herein described.

## EXAMPLE 14

5 Cupric stearate replaced the cadmium stearate of Example 12 in this example. Additionally, there was added to the mixture a small amount of sodium iodide, to prevent premature reaction and reduction of contrast. The sheet was light tan in color, changing rapidly to purple when heated to 75-85° C., and produced thermocopies having adequate contrast and detail.

## EXAMPLE 15

15 Thirty parts by weight of a dispersion of diphenyl carbazole in ten times its weight of heptane were mixed with 5 parts of a 5% solution of rubber in heptane and coated in a thin layer on flax tissue. Over the dried coating there was then applied a further coating of a mixture of 20 30 parts of a dispersion of zinc stearate in 5 times its weight of heptane, and 5 parts of the 5% rubber solution. The coated and dried sheet appeared snow white; it printed to a scarlet image at approximately 100° C.

20 The reactions employed in Examples 11-15 will be recognized as typical color reactions for the detection of the particular polyvalent metal ion employed. Many other reactions having similar applications are well known, having been published, for example, by Dr. F. Feigl in his book, "Qualitative Analysis by Spot Tests." The reactants selected must be solid at room temperatures, must be visibly inter-reactive at room temperatures when properly combined as by means of a mutual solvent, and at least one of the reactants must be fusible at a temperature within the range of about 60-120° C. The polyvalent metal ion is preferably introduced as the fusible salt of an organic acid, as shown in Examples 11-15; but other metallic compounds may be substituted where a fusible organic spot-test reagent, such as 2-nitroresorcinol (M. 83-85° C.) or 8-hydroxyquinoline (M. 75-76° C.), is to be used. Strongly colored, odorous, volatile, or light-sensitive reagents are generally undesirable but may be found useful for special purposes, particularly when introduced in the inner layer of structures as described in Example 15. Methyl cellulose and polyvinyl butyral are examples of additional suitable binders.

25 The reactive solid components are conveniently applied to paper or other supporting structure as a dispersion in a solution of a bonding agent in a suitable volatile vehicle, as disclosed in the above examples. The bonding agent assists in retaining the reactants on the surface of the support. However, other methods of applying the reactants to the supporting surface and of maintaining them in proper relationship thereon may alternatively be employed. For example, a polymerizable monomer may be substituted for the solution of bonding agent; after application, the monomer may be polymerized in situ to form a binder film. The powdered reactants may be dispersed within, or on the surface of, a fibrous web or other supporting structure in the substantial absence of any added bonding agent. Additionally, the use of a film-forming bonding agent, such for example as the nitrocellulose of Example 10 or other equivalent transparent film-forming binder, as a self-supporting film as well as a binder and carrier for the reactive ingredients is also contemplated. In this type of product, the film-forming composition containing the color-

producing reactants may be coated and dried on a temporary support, and the dry film subsequently removed by stripping to provide an exceedingly thin copying-paper. Compositions employing a reactant or reactants which are themselves film-forming, or which have adequate adhesion to a supporting web, ordinarily require no auxiliary bonding or film-forming agent.

Certain advantageous results may be obtained by proper selection and proportioning of the bonding agent as well as the reactants, and in our preferred compositions we therefore contemplate the use of a suitable inert bonding agent or combination of bonding agents in significant proportions. The degree of contrast obtainable with our copying-paper is readily controlled, for example, by suitably proportioning the relative amounts of binder and of reactants. Thus, increased contrast has been obtained by increasing the percentage of binder, and thereby presumably increasing the distance and the amount of non-reactive material between or around the individual particles of reactants. Conversely, a reduction in the percentage of bonding agent reduces the contrast and increases the detail obtainable in resultant copy.

Changes in the particle size and shape of any one or all of the reactant materials, and in the relative amounts of the individual reactants, will also have some effect on the results obtained. Stoichiometric relationships between reactants may in any cases be determined, but are not necessarily most advantageous. The proportions shown in the specific examples of the particular reactants therein disclosed have been found to produce good results, and may be used as a guide for the proper proportioning of other reactants; but many variations will be found to produce acceptable products and are here contemplated.

Where desired, various inert materials, such for example as pigments or the like, may be added to the sensitizing compositions of our invention. Additional surface coatings, e. g. of film-forming materials, may be applied as protective layers, or to impart desirable color, or for other purposes. Other modifications will be apparent.

In order to assure a clear understanding of the structure of our novel product and the manner in which it may be utilized, e. g. in the copying of printed matter, reference is made to the accompanying drawing, in which:

Figure 1 is a conventionalized and enlarged cross-section of one example of a suitable heat-sensitive coating on a supporting member;

Figures 2, 3, and 4 are perspective views (partially cut away) of three different arrangements of a printed surface in relation to the coated surface of the copying-paper in obtaining facsimile reproductions of printed or other graphic matter on the heat-sensitive coated copying-papers of this invention; and

Figure 5 is a diagrammatic, sectional view of one example of structure, including a suitable source of radiant energy, that may be employed for copying printed sheet material.

In Figure 1, a heat-sensitive layer 10, consisting of two finely-divided reactant materials 11 and 12, the individual solid particles of which are contained within a binder material 13, is supported on a supporting member 14.

In Figure 2, a transparent heat-sensitive copying-paper 15, consisting of a heat-sensitive layer 19 on a thin transparent backing 16 (both shown in cut-away section) is placed against a printed page 17, with the uncoated surface of the trans-

parent backing 16 in contact with the printed characters 18 of which a facsimile copy is desired. The transparent backing 16 of Figure 2 is a specific member of the class more generically represented in Figure 1 by supporting member 14. On exposure of the composite to intense illumination, as herein elsewhere explained, and in this case with the transparent heat-sensitive sheet 15 being between the source of light and the printed surface, a differential darkening, or other visible change, indicated by darkened area 19, is rapidly obtained in the heat-sensitive layer 10, corresponding to the printed character 18 therebelow.

The finished print obtained by the procedure outlined above in connection with Figure 2 is directly readable from the surface carrying the heat-sensitive layer. Transparency of the sheet material 15 to visible light is therefore not essential for subsequent reading of the copy obtained. Consequently the requirement of transparency here refers to the ability of the sheet to pass radiant energy of the wave-length employed in the copying process. The use of visible light thus imposes the requirement of "visible transparency," as manifested, for example, in the construction embodying cellophane and described under Example 1. With other wave-lengths, e. g. in the high-energy infra-red region, sheet material which is transparent to the infra-red but which may appear translucent or even opaque to the eye may be used and is here contemplated.

In Figure 3, the heat-sensitive layer 10 of the (visibly) transparent heat-sensitive copying-paper 15 is placed directly in contact with the printed characters 18 of the printed page 17. High intensity radiation directed against the transparent backing 16 results in a visible change, in the sensitive layer 10, corresponding to the printed characters 18, indicated by the darkened area 19 (partially concealed in the drawing). The resulting copy is a direct facsimile of the printed original when viewed through the visibly transparent backing 16.

In Figure 4, the heat-sensitive coating 10 is disposed, as shown in cut-away section, on a supporting member 14, which may be either transparent, translucent or opaque, but which should be at least reasonably non-conductive to heat. A thin opaque printed page 20, which may or may not carry printed characters on the under side, but which has printed characters 18, of which a copy is desired, on the outer side, is placed against the sensitive layer 10. Proper irradiation of the outer printed side of the printed page 20 results in the formation of a visible facsimile copy or darkened area 19, on the sensitive layer 10, corresponding to the printed characters 18, with no undesirable blurring or "ghost-image" formation being obtained from any similar printed characters which may be present on the under-side of the page 20.

In Figure 5, which illustrates in cross-section one means by which reproductions of printed matter may conveniently be made according to the principles set forth in connection with Figure 2, an electrically-activated high-intensity source of useful radiation such as light rays 23, comprising an incandescent line filament 21 in transparent evacuated envelope 22, is shown supported within a movable trough-like reflector 24 of elliptical cross-section. Filament 21 is located at one focal line of the elliptical reflector; consequently light rays 23, emanating therefrom, are focused at the other focal line, which is caused to coincide with the printed surface of printed

page 17, carrying printed or other graphic characters 18 of which a facsimile copy is desired.

Page 17 rests on the uncoated surface of a sheet of transparent heat-sensitive copying-paper 15, consisting of a transparent backing 16 and a heat-sensitive coating 10. The copying-paper rests on a transparent heat-insulating sheet material 25, which may be an open-mesh screen such as silk bolting-cloth, and this screen in turn rests on a transparent support 26, which may be a glass plate, preferably of heat-resistant glass. (Where support 26 is inherently sufficiently heat-non-conductive or is suitably roughened or otherwise treated at the surface so as to present a non-conductive surface to the copying-paper 15, the separate thickness of insulation 25 may be eliminated.) The copy-paper 15 and page 17 are held in close and heat-conductive contact by means of a heat-insulating cover 27, which may be a wooden cover, as shown in Figure 5, or may be constructed of any other suitable material including a soft and flexible material such as a pneumatic or hydraulic pressure-bag. If desired, the cover 27, and the underlying printed page 17, may be maintained at any desired temperature below the printing temperature of the copying-paper 15, by suitable temperature control means. The elliptical reflector 24, with its enclosed light source, is movable across the surface of the thermographic assembly, as indicated by the double arrow 28, by suitable means (not shown), in a plane such that the light rays 23 are continuously focused at the printed surface of the printed page 17. The rate of movement of the reflector assembly is adjustable, to compensate for differences in the thickness and heat conductivity of the page to be copied, here shown as printed page 17, and also to compensate for differences in the sensitivity of the temperature-sensitive layer 10, the intensity of light output, and various other factors.

For rapid copying of text-book pages, letters, or the like with the apparatus of Figure 5, it has been found convenient to use a 2000-watt coiled tungsten line-filament incandescent lamp, 10 inches long, with "Pyrex" glass envelope, mounted in an elliptical reflector 24. The resulting concentration of radiation is of such high intensity as to cause charring or burning if allowed to remain focused on the same section of paper for more than about one second. With this light source, and with temperature-sensitive copying-paper such as that described under the various examples, clear unfogged facsimiles may be obtained. However, many other sources of radiation, including ordinary high-intensity incandescent lamps, photoflash lamps, electric arc, infra-red lamps, concentrated sunlight, etc., have been found to be effective in various thermographic assemblies using our heat-sensitive copying-papers.

Many modifications, both in preparing the reactive compositions and the coated materials, and in utilizing the products in the direct reproduction of graphic subject-matter, have been described. While the importance of each of these and other modifications in the commercial application of the principles involved will become obvious in view of the foregoing description, it will be even more apparent that the underlying principle, on which the novel phenomena herein presented are based, remains the same in all of the applications and modifications thereof. This principle involves the selection and blending of two or more solid reactants in such a

manner that the reactants are prevented from combining or reacting with each other until the blend is heated to or above a predetermined range of temperature. When such a temperature is reached, however, the reactants are enabled rapidly to combine or react, whereupon there is produced a visible indication of such action, e. g. a color change. While the action thus obtained is of value under a wide variety of conditions, it has been shown to be particularly valuable in making available, as a new article of manufacture, a heat-sensitive copying paper suitable for the preparation of visible light-stable copies of graphic subject-matter by methods involving only the exposure of such matter to intense irradiation while in heat-conductive relationship with the heat-sensitive material.

Having now described our invention in terms of specific examples and embodiments, but without intent to be limited thereto, what we claim is as follows:

1. A heat-sensitive copying-sheet for making direct, high contrast, clear detail copies of graphic subject-matter as herein described, said copying-sheet being non-sticking at 120° C., being stable at normal room and storage temperatures, and being rapidly and permanently visibly changed when heated from room temperature to 120° C.; said copying-sheet comprising a support having low thermal conductivity, and a heat-sensitive layer firmly bonded thereto and containing a plurality of stable ionizable dissociable normally solid reactant materials including at least one electron donor component and at least one electron acceptor component disposed in contiguity with each other in said layer, at least one of said components being fusible at a temperature within the range of about 60-120° C. and being present in an amount such that on fusion and reaction with other components a visible change is produced in the heat-sensitive layer, said components being maintained in physically distinct and chemically inter-reactive relationship in said layer at normal room and storage temperatures, and said components being so selected as to be inter-reactive in a direct ion-exchange electron acceptor-donor chemical reaction at room temperature in a mutual solvent capable of permitting ionization of said components and with the formation of a stable, visibly distinct, highly polarized compound which is less dissociable than either of said components.

2. A heat-sensitive copying-sheet for making direct, high contrast, clear detail copies of graphic subject-matter as herein described, said copying-sheet being non-sticking at 120° C., being stable at normal room and storage temperatures, and being rapidly and permanently visibly changed when heated from room temperature to 120° C.; said copying-sheet comprising a support having low thermal conductivity, and a heat-sensitive layer containing, uniformly dispersed in a film-forming binder non-fusing at temperatures below about 120° C., a multitude of closely spaced solid particles of a plurality of stable ionizable dissociable normally solid reactant materials including at least one electron donor component and at least one electron acceptor component, at least one of said components being fusible at a temperature within the range of about 60-120° C. and being present in an amount such that on fusion and reaction with other components a visible change is produced in the heat-sensitive layer, said components being maintained in physically distinct and chemically inter-reactive

relationship in said layer at normal room and storage temperatures, and said components being so selected as to be inter-reactive in a direct ion-exchange electron acceptor-donor chemical reaction at room temperature in a mutual solvent capable of permitting ionization of said components and with the formation of a stable, visibly distinct, highly polarized compound which is less dissociable than either of said components.

3. The heat-sensitive copying-sheet of claim 1 wherein an electron acceptor component is an ionizable compound of an anion and a polyvalent metal cation, and an electron donor component is an ionizable organic reagent rapidly reactive with said polyvalent metal cation to provide a visibly distinct reaction product.

4. The heat-sensitive copying-sheet of claim 2 wherein an electron acceptor component is an ionizable compound of an anion and a polyvalent metal cation, and an electron donor component is an ionizable organic reagent rapidly reactive with said polyvalent metal cation to provide a visibly distinct reaction product.

5. A copying-sheet according to claim 1 in which an electron acceptor component is an iron salt melting at a temperature within the range of about 60-120° C., and an electron donor component is a water-insoluble organic compound having an iron cyanide complex ion.

6. A copying-sheet according to claim 5 in which the iron salt is a ferric salt of a fatty acid.

7. A copying-sheet according to claim 6 in which the electron donor component is a water-

insoluble organic reaction product of an organic amine and a water-soluble compound having an iron cyanide complex ion.

8. A copying-sheet according to claim 2 in which an electron acceptor component is an iron salt melting at a temperature within the range of about 60-120° C., and an electron donor component is a water-insoluble organic compound having an iron cyanide complex ion.

9. A copying-sheet according to claim 8 in which the iron salt is a ferric salt of a fatty acid.

10. A copying-sheet according to claim 9 in which the electron donor component is a water-insoluble organic reaction product of an organic amine and a water-soluble compound having an iron cyanide complex ion.

11. A copying-sheet according to claim 10 in which the electron donor component is a water-insoluble organic reaction product of an alkyl amine and a water-soluble ferrocyanide.

12. A copying-sheet according to claim 10 in which the electron donor component is a water-insoluble organic reaction product of an alkyl amine and a water-soluble ferricyanide.

CARL S. MILLER.  
BRYCE L. CLARK.

References Cited in the file of this patent

UNITED STATES PATENTS

| Number    | Name     | Date          |
|-----------|----------|---------------|
| 1,844,199 | Bicknell | Feb. 9, 1932  |
| 2,378,585 | Schroth  | June 19, 1945 |